



US011242614B2

(12) **United States Patent**  
**Curran et al.**

(10) **Patent No.:** **US 11,242,614 B2**  
(45) **Date of Patent:** **\*Feb. 8, 2022**

(54) **OXIDE COATINGS FOR PROVIDING CORROSION RESISTANCE ON PARTS WITH EDGES AND CONVEX FEATURES**

(71) Applicant: **Apple Inc.**, Cupertino, CA (US)

(72) Inventors: **James A. Curran**, Morgan Hill, CA (US); **Aaron D. Paterson**, Livermore, CA (US); **Brian M. Gable**, San Jose, CA (US)

(73) Assignee: **Apple Inc.**, Cupertino, CA (US)

(\*) Notice: Subject to any disclaimer, the term of this patent is extended or adjusted under 35 U.S.C. 154(b) by 252 days.

This patent is subject to a terminal disclaimer.

(21) Appl. No.: **15/881,305**

(22) Filed: **Jan. 26, 2018**

(65) **Prior Publication Data**

US 2018/0237936 A1 Aug. 23, 2018

**Related U.S. Application Data**

(60) Provisional application No. 62/460,691, filed on Feb. 17, 2017.

(51) **Int. Cl.**

**C25D 21/00** (2006.01)

**C25D 11/34** (2006.01)

(Continued)

(52) **U.S. Cl.**

CPC ..... **C25D 21/00** (2013.01); **C25D 11/04** (2013.01); **C25D 11/08** (2013.01); **C25D 11/12** (2013.01);

(Continued)

(58) **Field of Classification Search**

None

See application file for complete search history.

(56) **References Cited**

**U.S. PATENT DOCUMENTS**

2,692,851 A 10/1954 Burrows  
3,388,050 A 6/1968 Wainer et al.  
(Continued)

**FOREIGN PATENT DOCUMENTS**

CH 691064 A5 4/2001  
CN 1254028 A 5/2000  
(Continued)

**OTHER PUBLICATIONS**

Chinese Patent Application No. 201680050544.6—Second Office Action dated Sep. 27, 2019.

(Continued)

*Primary Examiner* — Humera N. Sheikh

*Assistant Examiner* — Elizabeth D Ivey

(74) *Attorney, Agent, or Firm* — Dorsey & Whitney LLP

**ABSTRACT**

Anodic oxide coatings that provide corrosion resistance to parts having protruding features, such as edges, corners and convex-shaped features, are described. According to some embodiments, the anodic oxide coatings include an inner porous layer and an outer porous layer. The inner layer is adjacent to an underlying metal substrate and is formed under compressive stress anodizing conditions that allow the inner porous layer to be formed generally crack-free. In this way, the inner porous layer acts as a barrier that prevents water or other corrosion-inducing agents from reaching the underlying metal substrate. The outer porous layer can be thicker and harder than the inner porous layer, thereby increasing the overall hardness of the anodic oxide coating.

**18 Claims, 9 Drawing Sheets**



# US 11,242,614 B2

Page 2

|                              |                                                                                                                                                   |                   |                  |                  |                   |           |
|------------------------------|---------------------------------------------------------------------------------------------------------------------------------------------------|-------------------|------------------|------------------|-------------------|-----------|
| (51) <b>Int. Cl.</b>         |                                                                                                                                                   |                   |                  |                  |                   |           |
| <i>C25D 11/30</i>            | (2006.01)                                                                                                                                         | 2009/0050485 A1   | 2/2009           | Wada et al.      |                   |           |
| <i>C25D 11/12</i>            | (2006.01)                                                                                                                                         | 2009/0152120 A1   | 6/2009           | Cao et al.       |                   |           |
| <i>C25D 11/04</i>            | (2006.01)                                                                                                                                         | 2009/0233113 A1   | 9/2009           | Hisamoto et al.  |                   |           |
| <i>C25D 11/16</i>            | (2006.01)                                                                                                                                         | 2010/0024534 A1   | 2/2010           | Li et al.        |                   |           |
| <i>C25D 11/08</i>            | (2006.01)                                                                                                                                         | 2010/0264036 A1   | 10/2010          | Hatanaka et al.  |                   |           |
| <i>C25D 11/24</i>            | (2006.01)                                                                                                                                         | 2010/0326839 A1   | 12/2010          | Morikawa et al.  |                   |           |
|                              |                                                                                                                                                   | 2011/0252874 A1   | 10/2011          | Patten et al.    |                   |           |
|                              |                                                                                                                                                   | 2011/0284383 A1   | 11/2011          | Cabot et al.     |                   |           |
|                              |                                                                                                                                                   | 2011/0297319 A1   | 12/2011          | Chen et al.      |                   |           |
|                              |                                                                                                                                                   | 2012/0000783 A1   | 1/2012           | Suda et al.      |                   |           |
|                              |                                                                                                                                                   | 2012/0103819 A1   | 5/2012           | Chang et al.     |                   |           |
|                              |                                                                                                                                                   | 2012/0298513 A1   | 11/2012          | Shimao et al.    |                   |           |
|                              |                                                                                                                                                   | 2013/0008796 A1   | 1/2013           | Silverman et al. |                   |           |
|                              |                                                                                                                                                   | 2013/0029094 A1   | 1/2013           | Chang et al.     |                   |           |
|                              |                                                                                                                                                   | 2013/0039773 A1*  | 2/2013           | Funk .....       | F01D 25/24        |           |
|                              |                                                                                                                                                   |                   |                  |                  | 416/223 R         |           |
| (52) <b>U.S. Cl.</b>         |                                                                                                                                                   |                   |                  |                  |                   |           |
| CPC .....                    | <i>C25D 11/16</i> (2013.01); <i>C25D 11/30</i> (2013.01); <i>C25D 11/34</i> (2013.01); <i>C25D 11/243</i> (2013.01); <i>C25D 11/246</i> (2013.01) | 2013/0008796 A1   | 1/2013           | Silverman et al. |                   |           |
|                              |                                                                                                                                                   | 2013/0029094 A1   | 1/2013           | Chang et al.     |                   |           |
|                              |                                                                                                                                                   | 2013/0039773 A1*  | 2/2013           | Funk .....       | F01D 25/24        |           |
|                              |                                                                                                                                                   |                   |                  |                  | 416/223 R         |           |
| (56) <b>References Cited</b> |                                                                                                                                                   |                   |                  |                  |                   |           |
| U.S. PATENT DOCUMENTS        |                                                                                                                                                   |                   |                  |                  |                   |           |
| C25D 11/18                   |                                                                                                                                                   |                   |                  |                  |                   |           |
| 3,411,994 A                  | 11/1968                                                                                                                                           | Wainer et al.     | 2013/0075262 A1  | 3/2013           | Teng              |           |
| 3,723,258 A                  | 3/1973                                                                                                                                            | Podell et al.     | 2013/0153427 A1  | 6/2013           | Tatebe            |           |
| 3,985,629 A                  | 10/1976                                                                                                                                           | Kimura            | 2013/0156635 A1  | 6/2013           | Lee et al.        |           |
| 4,039,355 A                  | 8/1977                                                                                                                                            | Takahashi et al.  | 2013/0302641 A1  | 11/2013          | Zhang et al.      |           |
| 4,066,516 A                  | 1/1978                                                                                                                                            | Sato              | 2013/0319866 A1  | 12/2013          | Browning et al.   |           |
| 4,189,360 A                  | 2/1980                                                                                                                                            | Woods et al.      | 2013/0319868 A1  | 12/2013          | Yoshida et al.    |           |
| 4,483,751 A                  | 11/1984                                                                                                                                           | Murayama et al.   | 2013/0319872 A1* | 12/2013          | Woodhull .....    | C25D 7/00 |
| 4,518,468 A                  | 5/1985                                                                                                                                            | Fotland et al.    |                  |                  | 205/120           |           |
| 4,606,796 A *                | 8/1986                                                                                                                                            | Hanazima .....    | 2014/0061054 A1  | 3/2014           | Ye                |           |
|                              |                                                                                                                                                   | 205/174           | 2014/0083861 A1  | 3/2014           | Askin et al.      |           |
| 4,631,112 A                  | 12/1986                                                                                                                                           | Usui et al.       | 2014/0166490 A1  | 6/2014           | Tatebe et al.     |           |
| 4,856,326 A                  | 8/1989                                                                                                                                            | Tsukamoto         | 2014/0190739 A1  | 7/2014           | Zhou et al.       |           |
| 4,894,127 A                  | 1/1990                                                                                                                                            | Wong et al.       | 2014/0262790 A1  | 9/2014           | Levendusky et al. |           |
| 4,987,766 A                  | 1/1991                                                                                                                                            | Brar et al.       | 2015/0029414 A1  | 1/2015           | Hur et al.        |           |
| 5,066,368 A                  | 11/1991                                                                                                                                           | Pasqualoni et al. | 2015/0090373 A1  | 4/2015           | Gable et al.      |           |
| 5,078,845 A                  | 1/1992                                                                                                                                            | Kunugihara et al. | 2015/0132541 A1  | 5/2015           | McDonald et al.   |           |
| 5,277,788 A                  | 1/1994                                                                                                                                            | Nitowski et al.   | 2015/0368515 A1  | 12/2015          | Lu et al.         |           |
| 5,336,341 A                  | 8/1994                                                                                                                                            | Maejima et al.    | 2016/0060783 A1  | 3/2016           | Curran et al.     |           |
| 5,472,788 A                  | 12/1995                                                                                                                                           | Benitez-Garriga   | 2016/0237586 A1  | 8/2016           | Curran et al.     |           |
| 5,705,225 A                  | 1/1998                                                                                                                                            | Dornfest et al.   | 2016/0289858 A1  | 10/2016          | Curran et al.     |           |
| 5,919,561 A                  | 7/1999                                                                                                                                            | Fuchs et al.      | 2016/0290917 A1  | 10/2016          | Hamann et al.     |           |
| 6,027,629 A                  | 2/2000                                                                                                                                            | Hisamoto et al.   | 2016/0312374 A1  | 10/2016          | Duffy et al.      |           |
| 6,235,409 B1                 | 5/2001                                                                                                                                            | Serafin et al.    | 2017/0051425 A1  | 2/2017           | Curran et al.     |           |
| 6,339,958 B1                 | 1/2002                                                                                                                                            | Tsui et al.       | 2017/0051426 A1  | 2/2017           | Curran et al.     |           |
| 6,581,446 B1                 | 6/2003                                                                                                                                            | Deneuville et al. | 2017/0088917 A1  | 3/2017           | Curran et al.     |           |
| 7,166,205 B2                 | 1/2007                                                                                                                                            | Kuo et al.        | 2017/0121837 A1  | 5/2017           | Tatebe et al.     |           |
| 7,527,872 B2                 | 5/2009                                                                                                                                            | Steele et al.     | 2017/0292202 A1  | 10/2017          | Curran et al.     |           |
| 7,732,056 B2                 | 6/2010                                                                                                                                            | Bhatnagar et al.  | 2018/0049337 A1  | 2/2018           | Curran et al.     |           |
| 7,820,300 B2                 | 10/2010                                                                                                                                           | Dolan             | 2019/0037721 A1  | 1/2019           | Curran et al.     |           |
| 8,016,948 B2                 | 9/2011                                                                                                                                            | Wang et al.       |                  |                  |                   |           |
| 8,145,411 B2                 | 3/2012                                                                                                                                            | Watanabe et al.   | CN 1616709 A     | 5/2005           |                   |           |
| 8,309,237 B2                 | 11/2012                                                                                                                                           | Levendusky et al. | CN 1632178 A     | 6/2005           |                   |           |
| 8,318,256 B2                 | 11/2012                                                                                                                                           | Ishii et al.      | CN 1774158 A     | 5/2006           |                   |           |
| 8,535,505 B2                 | 9/2013                                                                                                                                            | Yi et al.         | CN 1965618 A     | 5/2007           |                   |           |
| 8,691,403 B2                 | 4/2014                                                                                                                                            | Amakusa et al.    | CN 101048277 A   | 10/2007          |                   |           |
| 8,950,465 B2                 | 2/2015                                                                                                                                            | Lin et al.        | CN 101287861 A   | 10/2008          |                   |           |
| 8,962,163 B2                 | 2/2015                                                                                                                                            | Shimae et al.     | CN 101298690 A   | 11/2008          |                   |           |
| 8,968,548 B2                 | 3/2015                                                                                                                                            | Lai et al.        | CN 101325849 A   | 12/2008          |                   |           |
| 9,133,559 B2                 | 9/2015                                                                                                                                            | Silverman et al.  | CN 101970723 A   | 2/2011           |                   |           |
| 9,312,511 B2                 | 4/2016                                                                                                                                            | Mandlik et al.    | CN 102333897 A   | 1/2012           |                   |           |
| 9,349,536 B2                 | 5/2016                                                                                                                                            | Lee et al.        | CN 102654782 A   | 9/2012           |                   |           |
| 9,359,686 B1                 | 6/2016                                                                                                                                            | Curran et al.     | CN 102666894 A   | 9/2012           |                   |           |
| 9,512,510 B2                 | 12/2016                                                                                                                                           | Hatta             | CN 103484737 A   | 1/2014           |                   |           |
| 9,669,604 B2                 | 6/2017                                                                                                                                            | Tatsumi et al.    | CN 103484916 A   | 1/2014           |                   |           |
| 9,869,623 B2                 | 1/2018                                                                                                                                            | Hamann et al.     | CN 103526088 A   | 1/2014           |                   |           |
| 2003/0196907 A1              | 10/2003                                                                                                                                           | Viola             | CN 103732772 A   | 4/2014           |                   |           |
| 2004/0004003 A1              | 1/2004                                                                                                                                            | Hesse             | CN 103930600 A   | 7/2014           |                   |           |
| 2004/0115410 A1*             | 6/2004                                                                                                                                            | Nagaraj .....     | CN 103938250 A1  | 7/2014           |                   |           |
|                              |                                                                                                                                                   | 428/210           | CN 104762538 A   | 7/2015           |                   |           |
|                              |                                                                                                                                                   |                   | CN 108531958 A   | 9/2018           |                   |           |
| 2004/0129574 A1              | 7/2004                                                                                                                                            | Kia et al.        | EP 997545 A1     | 5/2000           |                   |           |
| 2005/0061680 A1              | 3/2005                                                                                                                                            | Dolan             | EP 1688020 B1    | 8/2006           |                   |           |
| 2005/0106403 A1              | 5/2005                                                                                                                                            | Yui               | EP 1397244 B1    | 12/2009          |                   |           |
| 2006/0019035 A1              | 1/2006                                                                                                                                            | Munz et al.       | EP 2301760 A2    | 3/2011           |                   |           |
| 2006/0086475 A1              | 4/2006                                                                                                                                            | Miyashita et al.  | EP 2817948 A1    | 12/2014          |                   |           |
| 2006/0108030 A1              | 5/2006                                                                                                                                            | Yoshioka et al.   | JP S4925538 B1   | 7/1974           |                   |           |
| 2006/0204780 A1              | 9/2006                                                                                                                                            | Vega et al.       | JP H0347937 A    | 2/1991           |                   |           |
| 2007/0000583 A1              | 1/2007                                                                                                                                            | Rioja et al.      | JP 2000313996 A  | 11/2000          |                   |           |
| 2008/0274375 A1              | 11/2008                                                                                                                                           | Ng et al.         | JP 2009209426 A  | 9/2009           |                   |           |
| 2008/0283408 A1              | 11/2008                                                                                                                                           | Nishizawa         | JP 2009209726 A  | 9/2009           |                   |           |
| 2009/0041988 A1              | 2/2009                                                                                                                                            | Ho et al.         | KR 20120021616 A | 3/2012           |                   |           |

(56)

## References Cited

## FOREIGN PATENT DOCUMENTS

|    |            |    |         |
|----|------------|----|---------|
| KR | 101235350  | B1 | 2/2013  |
| WO | 2010099258 | A1 | 9/2010  |
| WO | 2013123770 | A1 | 8/2013  |
| WO | 2013192579 | A1 | 12/2013 |
| WO | 2014045886 | A1 | 3/2014  |
| WO | 2014149194 | A1 | 9/2014  |
| WO | 2015199639 | A1 | 12/2015 |
| WO | 2018121212 | A1 | 7/2018  |

## OTHER PUBLICATIONS

International Search Report and Written Opinion for PCT Application No. PCT/US2015/025000 dated Jan. 26, 2016.

Garcia-Vergara, S. et al; "Morphology of enriched alloy layers in an anodized Al—Cu alloy" Applied Surface Science, 205 (2003),p. 121-127.

Alwitt, RS. and RC. McClung , "Mechanical Properties of Anodized Aluminum Coatings"; Proceedings of the SUR/FIN792, American Electroplaters and Surface Finishers Society, Atlanta, Georgia, Jun. 1992.

Yann Goueffon et al., "Study of Degradation Mechanisms of Black Anodic Films in Simulated Space Environment" URL:[http://webcache.googleusercontent.com/search?q=cache:fsJq5LjVTVII:esmal.esa.int/materials\\_news/isme09/of/6Contamination/S8%2520%2520Goueffon.pdf+&cd=1&hl=en&ct=clnk&gl=us](http://webcache.googleusercontent.com/search?q=cache:fsJq5LjVTVII:esmal.esa.int/materials_news/isme09/of/6Contamination/S8%2520%2520Goueffon.pdf+&cd=1&hl=en&ct=clnk&gl=us).

Henkel Corporation "Bonderite M-ED 9000 Anodizing Seal (Known as Anoseal 9000)" Technical Process Bulletin Issued Jun. 10, 2013.

Hao et al., "Sealing Processes of Anodic Coatings—Past, Present, and Future", Metal Finishing, vol. 98, Issue 12, Dec. 2000, p. 8-18.

International Search Report & Written Opinion for PCT Application No. PCT/US2015/010736 dated Oct. 29, 2015.

International Search Report & Written Opinion for PCT Application No. PCT/US2015/024349 dated Dec. 17, 2015.

International Search Report & Written Opinion for PCT Application No. PCT/US2014/053595 dated Jun. 24, 2015.

Habazaki et al., "Nanoscale Enrichments of Substrate Elements in the Growth of Thin Oxide Films", Corrosion Science, vol. 39, No. 4, pp. 731-737, 1997.

Vesborg et al., "Addressing the terawatt challenge: scalability in the supply of chemical elements for renewable energy," RSC Advances, 2, pp. 7933-7947, 2012.

European Patent Application No. 16150283.6—European Search Report dated Jun. 9, 2016.

International Patent Application No. PCT/US2016/043256—International Search Report and Written Opinion dated Oct. 12, 2016.

Diggle et al., Incorporation of anions: "Anodic oxide films on aluminum", Chemical Reviews, vol. 69, pp. 365-405 (1969), (41 Pages).

Charles Grubbs, "Anodizing of Aluminium", Metalfinishing, pp. 397-412, (16 Pages).

Milton Stevenson, "Anodizing", ASM Handbook vol. 5 (1994), 12 Pages.

Wang et. al., "Brilliant and tunable color of carbon-coated thin anodic aluminum oxide films", Appl. Phys. Lett., 91, 2007, 4 Pages.

Brock, et al., "European Coatings Handbook", 2000, Curt R. Vincentz, (pp. 374-376), 5 Pages.

Taiwanese Patent Application No. 105125817—Office Action and Search Report dated Apr. 19, 2017.

Achbach et.al. WADC technical report 55-150, Part VI, Project No. 7360, 1957.

Chinese Application for Invention No. 201610011395.4—First Office Action dated Jul. 21, 2017.

Saenz de Miera et. al. Surface and Interface Analysis, 2012 242, 241-246.

John C. Ion. Laser Processing of Engineering Materials. Elsevier, 2005 p. 160.

Chinese Application for Invention No. 201610202013.6—First Office Action dated Sep. 15, 2017.

Chinese Application for Utility Model No. 201490001542.4—First Office Action dated Sep. 27, 2017.

European Patent Application No. 16150283.6—Office Action dated Jan. 18, 2018.

Chinese Application for Utility Model No. 201490001542.4—Second Office Action dated Feb. 1, 2018.

Chinese Patent Application No. 201610011395.4—Second Office Action dated Feb. 14, 2018.

Guo Jialin etc., "Analysis of Effect on Hot Crackability of 6060 Alloy Oxide Film", Materials Research and Application, vol. 5, No. 3, p. 229-232.

Chinese Application for Invention No. 201610202013.6—Second Office Action dated Apr. 11, 2018.

Chinese Patent Application No. 201680050544.6—First Office Action dated Jan. 30, 2019.

Chinese Application for Invention No. 201610011395.4—Fourth Office Action dated Feb. 25, 2019.

Chinese Patent Application No. 201610011395.4—Third Office Action dated Aug. 15, 2018.

Habazaki, H. et al. Effects of Alloying Elements in Anodizing of Aluminium. Trans IMF, 1997, 75(1), 18-23. (Year: 1997), 6 pages.

The Aluminum Association, Inc. International Alloy Designations and Chemical Composition Limits for Wrought Aluminum and Wrought Aluminum Alloys. Jan. 2015. (Year: 2015), 38 pages.

Chinese Application for Invention No. 201610202013.6—Third Office Action dated Dec. 24, 2018.

Chinese Patent for Utility Model No. ZL201490001542.4—Utility Model Patent Evaluation Report (UMPER) dated Jan. 7, 2019.

Lee, W. et al., "Porous Anodic Aluminum Oxide: Anodization and Templated Synthesis of Functional Nanostructures", Chem. Rev. 2014, 15, 7487-7556, <https://doi.org/10.1021/cr500002z>, Jun. 13, 2014.

\* cited by examiner



*FIG. 1*



FIG. 2A

FIG. 2B



FIG. 3A

FIG. 3B



*FIG. 4A*



*FIG. 4B*



FIG. 5A



FIG. 5B



*FIG. 6A*



*FIG. 6B*



FIG. 6C



FIG. 6D



FIG. 6E



FIG. 7A



FIG. 7B



FIG. 8

## 1

**OXIDE COATINGS FOR PROVIDING  
CORROSION RESISTANCE ON PARTS WITH  
EDGES AND CONVEX FEATURES**

**CROSS REFERENCE TO RELATED  
APPLICATIONS**

This application claims the benefit of priority under 35 U.S.C. § 119(e) to U.S. Provisional Application No. 62/460, 691, entitled "OXIDE COATINGS FOR PROVIDING CORROSION RESISTANCE ON PARTS WITH EDGES AND CONVEX FEATURES," filed on Feb. 17, 2017, which is incorporated by reference herein in its entirety for all purposes.

Any publications, patents, and patent applications referred to in the instant specification are herein incorporated by reference in their entireties for all purposes. To the extent that the publications, patents, or patent applications incorporated by reference contradict the disclosure contained in the instant specification, the instant specification is intended to supersede and/or take precedence over any such contradictory material.

**FIELD**

The described embodiments relate to oxide films and methods for forming the same. The oxide films can have layered structures that provide improved adhesion.

**BACKGROUND**

When a metal part having convex edges or protruding features is anodized, the resulting anodic oxide film can exhibit small cracks along the convex edges and protruding features. These cracks can compromise the protective nature of the oxide film by providing pathways for water or other corrosion-inducing agents to reach the underlying metal part, thereby leaving the metal part susceptible to corrosion.

Certain high-strength aluminum alloys suffer from poor oxide adhesion when anodized. Alloying elements such as zinc accumulate at the interface between the metal and the oxide, and when combined with sulfur from the anodizing electrolyte, the zinc weakens the adhesion of the oxide. Regions of the oxide coating thus chip off relatively easily when mechanical stress is applied through incidents such as surface impacts. These chips expose the substrate, compromising the protective nature of the oxide film by providing pathways for water or other corrosion-inducing agents to reach the underlying metal part, thereby leaving the metal part susceptible to corrosion. The chips also constitute obvious cosmetic defects. What are needed therefore are improved anodic oxide films and anodizing techniques.

**SUMMARY**

This paper describes various embodiments that relate to oxide coatings useful for coating and preventing corrosion of metal substrates, including substrates having convex surface features. In particular embodiments, the oxide coatings include a porous corrosion-prevention layer proximate to the substrate.

According to some embodiments, a process for anodizing a metal substrate having a convex surface geometry, is described. The process can include converting a first amount of the metal substrate to a first metal oxide layer under a tensile strain condition that corresponds to a first electrical parameter, where the first metal oxide layer includes an

## 2

interstice that is capable of extending at least partially through the first metal oxide layer. The process can further include converting a second amount of the metal substrate that is overlaid by the first metal oxide layer to a second metal oxide layer under a compressive stress condition that corresponds to a second electrical parameter, where the second metal oxide layer (i) is located between the first metal oxide layer and a remaining portion of the metal substrate, and (ii) prevents the interstice from extending to the remaining amount of the metal substrate.

According to some embodiments, a part is described. The part can include a metal substrate having a convex surface geometry and a metal oxide coating disposed on the metal substrate. The metal oxide coating can include a first oxide layer having an interstice that is dependent upon the convex surface geometry, where the interstice extends at least partially through the first oxide layer. The metal oxide coating can further include a second oxide layer disposed between the first oxide layer and the metal substrate, where an interface that separates the second oxide layer from the metal substrate is generally free of an aggregated amount of alloying agents, thereby preventing the interstice from extending into the second oxide layer.

According to some embodiments, a method for improving interfacial adhesion between a metal substrate and a metal oxide layer formed on the metal substrate, the metal oxide layer including an inner oxide layer and an outer oxide layer disposed on the inner oxide layer, is described. The method can include forming the outer oxide layer by exposing a first portion of the metal substrate to an electrolyte under a tensile strain condition that corresponds to a first amount of a current density and forming the inner oxide layer by exposing a second portion of the metal substrate to the electrolyte under a compressive stress condition that corresponds to a second amount of the current density that is less than the first amount of the current density, thereby minimizing alloying agents from aggregating at an interface between the metal substrate and the inner oxide layer.

These and other embodiments will be described in detail below.

**BRIEF DESCRIPTION OF THE DRAWINGS**

The disclosure will be readily understood by the following detailed description in conjunction with the accompanying drawings, wherein like reference numerals designate like structural elements.

FIG. 1 shows perspective views of devices having metal surfaces that can be treated with the coatings described herein.

FIGS. 2A-2B and 3A-3B illustrate cross-section views of parts having geometric features that are prone to corrosion.

FIGS. 4A and 4B illustrate cross-section views of enclosures having geometric features that are prone to corrosion.

FIGS. 5A and 5B show cross-section views of a part undergoing anodizing processes for forming a corrosion-resistant oxide coating, in accordance with some embodiments.

FIGS. 6A-6E show cross-section views of portions of the part in FIGS. 5A-5B having the corrosion-resistant oxide coating.

FIGS. 7A and 7B show scanning electron microscope (SEM) images of cross-section views of a part having a corrosion-resistant oxide coating, in accordance with some embodiments.

FIG. 8 shows a flowchart indicating a process for forming a corrosion-resisting oxide coating, in accordance with some embodiments.

## DETAILED DESCRIPTION

Reference will now be made in detail to representative embodiments illustrated in the accompanying drawings. It should be understood that the following descriptions are not intended to limit the embodiments to one preferred embodiment. To the contrary, it is intended to cover alternatives, modifications, and equivalents as can be included within the spirit and scope of the described embodiments as defined by the appended claims.

Anodic oxide films that provide improved protection against corrosion for substrates having protruding features are described. The protruding features can include edges, corners, convex-shaped surfaces, and junction regions between non-parallel surfaces of a substrate. When a substrate having protruding features is anodized using conventional anodizing processes, the resulting oxide film can have cracks, interstices, gaps, or channels at areas covering the protruding features. This is because anodizing is a conversion process, whereby the oxide film is grown out of and into the substrate, resulting in an overall expansion of the outer surface of the oxide film. A protruding feature on the substrate generates an effective in-plane tensile strain in the oxide film during the anodizing process, which can cause cracks to form within the oxide film that compromise the protective nature of the oxide film.

The oxide films described herein include an inner oxide layer adjacent the substrate that is resistant to developing cracks, interstices, gaps, or channels during the anodizing process, even at high stress locations such as protruding features of the substrate. The inner oxide layer is formed under compressive stress conditions that counter the effective tensile strain induced by the protruding feature geometry. In this way, the inner oxide layer can form without cracks, interstices, gaps, or channels, thereby providing full coverage of the substrate and minimizing or eliminating corrosion. According to some embodiments, a thicker and harder outer oxide layer is formed over the inner oxide layer, thereby increasing the overall hardness of the oxide film.

According to some embodiments, methods for forming the oxide films include a two-phase anodizing process, with the second phase conducted using lower current density or lower voltage to generate the compressive stress conditions. For a feature having a given convex radius, the oxide films formed using the two-phase process show a far lower incidence of cracks, interstices, gaps, or channels compared to conventional oxide films.

As described herein, the term convex surface geometry can refer to a surface of a substrate (e.g., anodic oxide layer) that curves and extends outwards and away from a base portion of the same substrate. The convex surface geometry can include a radius of curvature, where cracks or convex surface geometry dependent interstices tend to form when the radius of curvature is greater than a threshold radius of curvature. In other words, the convex surface geometry can appear "more convex" when there is an increase in the radius of curvature and/or a greater change in the radius of curvature; thereby, increasing a tendency of the substrate to form cracks and channels. Additionally, these cracks and interstices are more likely to form in the surface of the substrate when the surface is subject to tensile strain, such as during an anodization process. For example, during the anodization process, the radius of curvature of a surface of the anodic

oxide layer is necessarily greater than a radius of curvature of the underlying substrate that was oxidized, which can induce lateral expansion of the anodic oxide layer. In other examples, these cracks and interstices can tend to form when the radius of curvature is less than 0.5 mm.

In some examples, the convex surface geometry can include surfaces (e.g., planar surfaces) that meet at an edge, where the edge can represent an abrupt change in the radius of curvature and represent a focal point for the formation of the interstice or the crack. In such some examples, the convex surface geometry can include an angle associated with where the planar surfaces meet. Cracks, fissures, and interstices that are dependent upon the convex surface geometry may tend to form when the angle at which the planar surfaces meet is less than a threshold angle. In other words, there is a greater tendency to form cracks, interstices, and channels when the angle between the surfaces is more acute (i.e., less than 90 degrees). In some examples, an acute angle between multiple surfaces may correspond to a sharp edge or a sharp protruding feature, and where further decreasing the acute angle between these multiple surfaces can lead to a sharper edge or a sharper protruding feature. In some examples, the sharpness of the edge or protruding feature can be based on the acute angle and/or the thickness of the surfaces.

As described herein, the terms oxide, anodic oxide, metal oxide, etc. can be used interchangeably and can refer to suitable metal oxide materials, unless otherwise specified. Furthermore, the terms coating, layer, film, etc. can be used interchangeably and can refer to any suitable material that covers a surface of a substrate, part, etc. unless otherwise specified. For example, an oxide formed by anodizing an aluminum or aluminum alloy substrate can form a corresponding aluminum oxide film, layer or coating.

The oxide coatings described herein are well suited for providing cosmetically appealing and protective surfaces to consumer products. For example, the oxide coatings can be used to form durable and cosmetically appealing finishes for housing of computers, portable electronic devices, wearable electronic devices, and electronic device accessories, such as those manufactured by Apple Inc., based in Cupertino, Calif.

These and other embodiments are discussed below with reference to FIGS. 1-8. However, those skilled in the art will readily appreciate that the detailed description given herein with respect to these Figures is for explanatory purposes only and should not be construed as limiting.

The methods described herein can be used to form durable and cosmetically appealing coatings for metallic surfaces of consumer electronic products, such as computing devices shown in FIG. 1, which includes portable phone 102, tablet computer 104, smart watch 106 and portable computer 108. Electronic devices 102, 104, 106 and 108 can each include housings that are made of metal or have metal sections. Aluminum alloys and other anodizable metals and their alloys can be used due to their ability to anodize and form a protective anodic oxide coating that protects the metal surfaces from scratches. Aluminum alloys, such as 5000 series, 6000 series or 7000 series aluminum alloys, may be choice metal materials due to their light weight and durability.

Products such as electronic devices 102, 104, 106 and 108 can include metal edges, corners and other geometric features that can be susceptible to corrosion and developing cosmetic defects when anodized using conventional techniques. This is, in part, because anodizing is a conversion process that consumes surface portions of a part. To illus-

trate, FIGS. 2A-2B and 3A-3B show cross-section views of parts, which are treated using a conventional anodizing process.

FIG. 2A shows part 200, which includes metal substrate 202 having a square shape with corners 203 and side defined by length  $a$ . FIG. 2B shows metal substrate 202 after a conventional anodizing process, where the metal substrate has a reduced length  $a'$ . Anodizing is a conversion process, whereby a portion of metal substrate 202 is consumed and converted to a corresponding oxide film 204 having thickness  $t$ . Dashed line 205 indicates the dimensions of the original surface of metal substrate 202 prior to the anodizing process. As shown, oxide film 204 grows into and out from the original surface of the metal substrate 202 by about  $t/2$ , and increases the length of part 300 to about  $a'+2t$ . This inherent expansion from the anodizing process induces tensile strain on oxide film 204. Since anodizing converts metal substrate 202 to a lower density porous oxide film 204, the inherent expansion which might be expected to accommodate some of this effective strain. However, this is balanced by mass loss (e.g., aluminum dissolving into the anodizing solution) and is largely expressed in an out-of-plane direction. Thus, those portions of oxide film 204 on corners 203 can experience significant in-plane tensile strain that causes channels 207 to form during the anodizing process. The likelihood of forming cracks or interstices and the width of channels 207 are functions of the angle of corners 203, with more acute angles associated with a higher likelihood of forming channels 207 and wider channels 207. In particular, the angle of corners can refer to convex surface geometrical features that refer to a portion of the oxide film 204 that protrudes or extends away from the oxide film 204. In other words, every internal angle of the convex surface geometrical features is less than or equal to 180 degrees. The angle of corners can refer to multiple surfaces that intersect or meet at a point. As the angle of the corner decreases (i.e., becomes more acute), then the corner becomes sharper and the amount of tensile strain induced at the oxide film 204 is increased. Consequently, increasing the amount of tensile strain at the oxide film 204 can cause channels 207 to form at the focal point where the multiple surfaces intersect. The likelihood of forming channels 207 and the width of the channels 207 can also depend on the thickness  $t$  of oxide film 204, with greater thicknesses associated with a higher likelihood of cracking or forming interstices, and with the width of channel 207 can be calculated at about  $t/V2$ .

FIG. 3A shows part 300, which includes metal substrate 302 having a radius  $r$  and a round shape defined by diameter  $2r$  and circumference  $2\pi r$ . FIG. 3B shows metal substrate 302 after a conventional anodizing process, whereby a portion of metal substrate 302 is consumed and converted to a corresponding oxide film 304 having thickness  $t$ . Subsequent to the anodization process, the metal substrate 302 has a reduced radius  $r'$ . Dashed line 305 indicates the dimensions of the original surface of metal substrate 302 prior to the anodizing process. Oxide film 304 grows into and out from original surface of the metal substrate 302 and expands the diameter of part 300 to about  $2r'+2t$  and expands the outer circumference of part 300 to about  $2\pi(r'+t)$ , which induces tensile strain on oxide film 304 that causes channel 307 to form. The likelihood of cracking or forming channels and the width of channel 307 are functions of the radius of curvature of substrate 302, with smaller radius of curvatures associated with a higher likelihood of cracking and forming channels, and forming a wider channel 307. The likelihood of forming channels and the width of the channels 307 are functions of the radius of curvature. In particular, the radius

of curvature of the oxide film 304 can refer to convex surface geometrical features (e.g., external surface features) that protrude or extend away from a base portion (e.g., inner surface) of the oxide film 304. In other words, the inner surfaces of the oxide film 304 are convex because the distance between two or more points of the oxide film 304 is the length of the shortest arc connecting them. As the radius of curvature increases and/or there is a greater increase in the amount of change in the radius of curvature, 10 can result in an increase the tendency of the oxide film 304 to form channels 307. Additionally, during the anodization process, the oxide film 304 necessarily has a greater radius of curvature than the underlying substrate 302. Therefore, the anodization process can lead to increased lateral expansion 15 of the oxide film 304, which can lead to formation of channels 307. The likelihood of cracking and forming channels, and the width of channel 307 can also depend on the thickness  $t$  of oxide film 304, with greater thicknesses associated with a higher likelihood of cracking and a wider channel 307.

FIGS. 4A and 4B illustrate cross-section views of enclosures having geometric features that, when anodized using convention processes, can cause channels to form within the resultant oxide film. FIG. 4A shows enclosure 400, which 25 includes metal substrate 402 having edge 403. The geometric constraints of edge 403 induce tensile stress within oxide coating 404 during the anodizing process, thereby causing channel 407 to form similar to as described above with 30 reference to FIGS. 2A-2B and 3A-3B. The size (e.g., as measured by width  $w$ ) of channel 407 will depend, in part, on the acuteness of edge 403 and thickness  $t$  of oxide coating 404. In some cases, width  $w$  of channel can range between about 10 micrometers to about 800 micrometers.

Although channel 407 may in some cases be too small to 35 be visible, channel 407 can act as a pathway for water, other corrosion-inducing agents, or other contaminant to reach underlying substrate 402, thereby compromising the protective nature of oxide coating 404. In some products, smaller channel 407 may not lead to significant corrosion of the 40 underlying substrate 402. Furthermore, the product may not be exposed to moisture on a regular basis during normal use. However, some products, such as some portable electronic devices, may be exposed to more aggressively corrosive environments, such as exposure to sweat, humid conditions, and chlorides from chlorinated or ocean water, which can exacerbate the corrosion process and lead to significant corrosion of substrate 402.

Furthermore, some types of metal substrates may be more 45 susceptible to corrosion. For example, some aluminum alloys that include relatively high levels of zinc may be more susceptible to corrosion than other aluminum alloys under certain conditions. In general, zinc can be added as an alloying element to increase the strength and hardness of an aluminum alloy. For example, some 7000-series aluminum 50 alloys (per The International Alloy Designation System), which are known for their high strength, can have relatively high levels of zinc. In some applications, the target yield strength for substrate 402 is at least about 330 MPa. In some cases, this corresponds to an aluminum alloy having a zinc 55 concentration of at least about 4 weight %. In other cases, this corresponds to an aluminum alloy having a zinc concentration of at least about 2 weight %. It is believed that zinc combines with magnesium as another alloying element to form precipitates such as  $MgZn_2$  (the  $\eta'$  or "eta-prime" phase), which gives the aluminum alloy its high strength. 60 Thus, the aluminum alloys having relatively high levels of zinc may also have relatively high levels of magnesium.

Despite the advantage of increasing the strength of the substrate, higher levels of zinc can also be associated with increased vulnerability to corrosion. Thus, the presence of channel 407 can be especially detrimental to those substrates 402 composed of aluminum alloys having zinc concentrations of about 4 weight % or higher.

It should be noted that width w of channel 407 can be on the order of micrometers, and is therefore generally three to four orders of magnitude greater than diameters of the pores formed within oxide coating 404 during the anodizing process, which are typically in the scale of tens of nanometers. Thus, a subsequent hydrothermal sealing process would not be able to sufficiently close off channel 407.

It should also be noted that a polymer coating applied over oxide coating 404 and into channel 407 used mitigate corrosion can detract from the tactile and visible cosmetics of oxide coating. In particular, a polymer coating may have a warm and sticky feeling compared to a cool and smooth feeling of an outer oxide coating. Furthermore, polymer coatings may introduce their own reliability limits, such as increased changes of discoloration under ultraviolet light exposure, or attack by certain everyday household chemicals.

FIG. 4B shows enclosure 420, which includes metal substrate 422 having a curved surface 423, which can correspond to a curved edge, a curved corner, or a curved protruding feature of enclosure 420. Oxide coating 424 formed using a conventional anodizing process includes channel 427. As described above with reference to FIG. 4A, channel 427 can act as a pathway for corrosion-inducing agents to reach metal substrate 422. Width w of channel 427 will depend, in part, on the radius of curvature of curved surface 423 and thickness t of oxide coating 424. For example, in some cases, radius of curvatures of about 0.5 mm or smaller for oxide coating 424 having thickness t of about 8 micrometers or greater can cause channel 427 to form. In some applications, thicknesses t of about 12 micrometers or greater may be preferred for adequate corrosion protection of some types of aluminum alloys. Thus, such oxide coatings would likely develop channels along convex geometrical surfaces or convex protruding features.

Described herein are anodizing methods for forming an oxide coating that provides improved corrosion resistance, especially useful on parts with edges, corners and convex features. Even a coarse blast texture, or a surface roughened through a laser marking or engraving procedure could result in such features. FIGS. 5A and 5B show cross-section views of part 500 undergoing an anodizing process in accordance with some embodiments. At FIG. 5A, metal substrate 502 of part 500 has undergone a first anodizing process, whereby a portion of substrate 502 is converted to first oxide layer 504. In some embodiments, substrate 502 corresponds to a metal portion of an enclosure of an electronic device, such as device 102, 104, 106 or 108, described above. Substrate 502 can be composed of any suitable anodizable material, including aluminum and aluminum alloys. In some embodiments, substrate 502 is composed of high-strength aluminum alloy, such as those having relatively high levels of zinc as an alloying element. As described above, higher concentrations of zinc and/or magnesium can be associated with greater yield strength and hardness. In some embodiments, substrate 502 is composed of an aluminum alloy having a zinc concentration of at least about 4 weight %. In some embodiments, substrate 502 is composed of an aluminum alloy having a zinc concentration of at least about 2 weight %. In some embodiments, substrate 502 is composed of an aluminum alloy having a magnesium concentration of at

least about 2 weight %. In some embodiments, substrate 502 is composed of an aluminum alloy having a magnesium concentration of at least about 1 weight %. In some applications, substrate 502 has a yield strength of at least about 330 MPa.

Another consideration regarding substrate 502 relates to the cosmetics. Color and finish quality can be important aspects when manufacturing consumer products. Some alloying elements, such as iron, copper, and silver, within substrate 502 can discolor first oxide layer 504. For example, copper can add a yellow color to the first oxide layer 504, which can be noticeable even when copper is added in quantities as low as about 0.2 weight %. Thus, in some embodiments, where such yellowing in first oxide layer 504 is undesirable, substrate 502 is composed of an aluminum alloy having a copper concentration of no more than about 0.2 weight %—in some embodiments, a copper concentration of no more than about 0.1 weight %. These and other details as to how alloying elements can affect strength and coloration of substrate 502 are described in U.S. patent application Ser. Nos. 14/830,699 and 14/830,705, both filed on Aug. 19, 2015, and U.S. patent application Ser. No. 14/927,225, filed on Oct. 29, 2015, each of which is incorporated herein in its entirety for all purposes.

Any suitable anodizing process can be used to form first oxide layer 504. In some embodiments, a “Type II anodizing” process (as defined by military specification MIL-A-8625 standards) is used, which involves anodizing in an aqueous sulfuric acid-based electrolyte. In some embodiments, the Type II anodizing process involves using an applied current density of between about 1 A/dm<sup>2</sup> and about 2 A/dm<sup>2</sup>. In a particular embodiment, the applied current density is no less than about 1.3 A/dm<sup>2</sup>. In some embodiments, the Type II anodizing involves using an electrolyte temperature of between about 15 degrees C. and about 25 degrees C. It should be noted that anodizing processes using other types of electrolytes might be used, including those using oxalic acid-based electrolytes or phosphoric acid-based electrolytes. However, sulfuric acid-based electrolytes can provide porous (and therefore dyeable), relatively colorless, and relatively durable coatings, which can be desirable characteristics for consumer products, such as electronic devices 102, 104, 106 and 108 described above.

First oxide layer 504 is porous in that it includes pores 505, which are formed during the anodizing process and which can be filled with colorant in a subsequent anodic film coloring operation. The size of pores 505 within first oxide layer 504 will vary depending on the anodizing process conditions. In some embodiments, pores 505 have diameters ranging between about 10 nanometers and about 50 nanometers. The thickness 506 of first oxide layer 504 can vary, depending on application requirements. In some consumer electronic enclosure applications, thickness 506 should be sufficiently large to provide adequate protection to substrate 502 against denting and scratching under normal use, and sufficiently small such that first oxide layer 504 remains cosmetically appealing and relatively colorless. In some embodiments, this corresponds to thickness 506 ranging between about 10 micrometers and about 50 micrometers. In some embodiments, this corresponds to thickness 506 ranging between about 10 micrometers and about 20 micrometers.

FIG. 5B shows part 500 after a second anodizing process is performed, whereby another portion of substrate 502 is converted to second oxide layer 508, having a thickness 510. Because of their relative positions, second oxide layer 508 can be referred to as an inner oxide layer and first oxide layer

can be referred to as an outer oxide layer. Together, first oxide layer 504 and second oxide layer 508 can be referred to as oxide coating 511, having a thickness 512 (thickness 506 plus thickness 510).

The second anodizing process is different than the first anodizing process used to form first oxide layer 504, in that the second anodizing process involves growing second oxide layer 504 under compressive stress conditions compared to tensile stress conditions of the first anodizing process. As described above with reference to FIGS. 2A-2B, 3A-3B and 4A-4B, oxide films grown under tensile stress can form interstices, cracks or channels, especially in those regions of a substrate that include high strain regions such as edges, corners and convex-shaped features. The second anodizing process involves adjusting anodizing parameters such that second oxide layer 508 experiences a compressive stress during its formation, so that it can tolerate a higher level of strain during its formation. Thus, second oxide layer 508 is less likely to develop channels compared to first oxide layer 504, even at high strain regions of a part, such as edges, corners, convex-shaped protrusions, or textured or roughened surfaces which exhibit sufficiently small radius of curvature or acute angles where different surfaces meet at an edge. This means that even if first oxide layer 504 has channels formed during the first anodizing process, second oxide layer 508 can remain crack-free or interstice-free and therefore protect substrate 502 from exposure to water, other corrosion-inducing agents, or other contaminant. These aspects will be described in detail below with reference to FIGS. 6A-6D.

Process conditions of the second anodizing process can vary. In some embodiments, the second anodizing process involves keeping part 500 in the same electrolyte as used during the first anodizing process, and reducing the current density compared to that used during the first anodizing process. One of the advantages of keeping part 500 in the same electrolyte during the first and second anodizing processes is that this simplifies manufacturing. In particular embodiments, the first and second anodizing processes are both performed in an aqueous sulfuric acid electrolyte (e.g., a 200 g/l solution at 25 degrees C.) and the current density is reduced by a factor of four (e.g., from about 1.6 A/dm<sup>2</sup> to about 0.4 A/dm<sup>2</sup>), corresponding to a reduction in voltage of about one half (½). In some embodiments, the second anodizing process involves using a current density ranging less than about 0.8 A/dm<sup>2</sup>. In a particular embodiment, the second anodizing process involves using a current density ranging between about 0.2 A/dm<sup>2</sup> and about 0.9 A/dm<sup>2</sup>. In another embodiment, the second anodizing process involves using a voltage ranging between about 6 volts and about 10 volts. In some embodiments, using a higher electrolyte temperature drops the effective voltage, thereby inducing a compressive stress conditions during the second anodizing process. In another variation, the current density (or voltage) is dropped as a continuous gradient and ends at a target low current density (or voltage) rather than abruptly dropped in one step.

Due to the different anodizing conditions, second oxide layer 508 has different structural properties than first oxide layer 504. The structural difference, which can be key to the present embodiments, is the stress during layer formation, with the second layer being formed under compressive stress. In particular, pores 518 within second oxide layer 508 are generally smaller in diameter compared to pores 505 of first oxide layer 504. In some embodiments, the diameters of pores 518 of second oxide layer 508 are about half (½) the diameters of pores 505 of first oxide layer 504. Thus, a first

pore in the first oxide layer 504 can have a first diameter that is greater than that of a pore in the second oxide layer 508 (e.g., the second diameter can be at least half the first diameter).

5 An undesirable consequence of anodizing conditions selected to induce compressive stress in the second oxide layer 508 (namely lower current density, lower voltage or higher electrolyte temperature) can be that reductive dissolution is greater. It can be a relatively "soft" anodizing 10 process, which results in softer oxide films. This softening particularly affects outer surface 516, and the outer portion of the first oxide layer 504, making the overall film less abrasion resistant. Thus, for those applications where the oxide coating hardness should be sufficiently high to resist 15 scratching and denting, the relatively "hard" process used to grow the first oxide layer 504 should constitute as much of the overall processing time as possible. The corresponding layer thickness 506 of first oxide layer 504 will be much greater than the layer thickness 510 of the second oxide layer 20 508. For example, in some consumer electronic enclosure applications where the oxide coating hardness should be sufficiently high to resist scratching and denting, the harder first oxide layer 504 should have a much greater thickness 506 compared to thickness 510 of the softer second oxide 25 layer 508. For example, in some consumer electronic enclosure applications, oxide coating 511 should have a hardness of at least about 250 HV<sub>0.05</sub> as measured in accordance with Vickers hardness testing standards—in some embodiments at least about 300 HV<sub>0.05</sub>. In some embodiments, thickness 30 510 of second oxide layer ranges between about 2% and about 15% of the thickness of oxide coating 511. In some embodiments, second oxide layer 508 has a thickness no greater than about 2 micrometers. In some consumer product applications, thickness 512 of oxide coating 511 should be 35 at least about 8 micrometers in order to provide adequate protection to substrate 502, but not be so thick as to negatively affect the cosmetics of part 500. In particular embodiments, thickness 512 ranges between about 8 micrometers and about 30 micrometers. In a particular embodiment, thickness 512 ranges between about 10 micrometers and about 15 micrometers.

In addition to being generally crack-free or interstice-free due to the compressive stress conditions of the second anodizing process, the presence of second oxide layer 508 45 can provide other advantages. For example, second oxide layer 508 can better adhere to substrate 502 compared to first oxide layer 504 due to the compressive stress conditions from which second oxide layer 508 was formed. This means that oxide coating 511 can be less susceptible to delamination 50 compared to an oxide coating having only first oxide layer 504. Thus, part 500 would be less susceptible to chipping or delamination that would cause cosmetic defects and also leave those chipped or delaminated areas of substrate 502 exposed and vulnerable to corrosion.

55 Another way in which second oxide layer 508 can provide structural advantages to oxide coating 511 relates to interface 514 between first oxide layer 504 and second oxide layer 508. In particular, oxide coating 511 may be subjected to forces that impact outer surface 516 during use of part 60 500, such as from scratching, gouging or drop events, which can cause damage in the form of channels within oxide coating 511. If these post-anodizing channels occur, they may propagate through first oxide layer 504 and be deflected in a lateral direction (generally parallel to outer surface 516) 65 by interface 514, thereby preventing such channels from propagating through second layer oxide layer 508. It should be noted that this type of channel occurs during the use of

## 11

part 500 (i.e., after oxide coating 511 has already been formed), whereas channels 207 and 407 described above with reference to FIGS. 2A-2B, 3A-3B and 4A-4B occur during the anodizing process. In this way, second oxide layer 508 can provide protection against post-anodizing channels. It should be noted that, in some embodiments, thickness 510 of second oxide layer 508 is at least a prescribed minimum thickness in order to prevent or reduce the likelihood of such post-anodizing channels. In some embodiments, this minimum thickness is about 0.5 micrometers. Thus, in some embodiments, thickness 510 ranges between about 0.5 micrometers and about 2 micrometers.

In particular, the presently described two-step anodizing process provides a means of improving the interfacial adhesion between an anodic oxide coating and relatively pure 7000-series aluminum alloys comprising zinc. For instance, specific types of aluminum alloys (e.g., aluminum-zinc alloys, aluminum-magnesium alloys, etc.) can be susceptible to delamination when anodized using a conventional Type II anodizing process. In particular, specific types of electrolytes, such as sulfuric acid, can include chemical species (e.g., sulfur) that preferentially combine with alloying agents (e.g., zinc) to form delamination compounds that can promote delamination between the oxide coating 511 and the substrate 502. In order to minimize the possibility of delamination of these parts during the anodization process, other types of acids, such as oxalic acid and mixed acids can be generally used. However, these types of acids are associated with certain drawbacks, such as a higher probability of discoloring these parts with a yellow appearance during the anodization process. Consequently, the discoloration of these anodized parts is cosmetically unappealing.

Beneficially, the techniques described herein are able to improve interfacial adhesion between the oxide coating 511 and the substrate 502 relative to the conventional Type II anodizing process, such that these parts can be anodized using electrolytes, such as sulfuric acid, which were previously avoided due to their strong likelihood of inducing delamination. Additionally, by anodizing these parts using these types of electrolytes, discoloration of these parts can be generally avoided.

According to some embodiments, interfacial adhesion between the oxide coating 511 and the substrate 502 can be improved by subjecting the part 500 to a two-step anodizing process, where first and second steps for forming the first metal oxide coating 504 and the second metal oxide coating 508 are performed under different electrical parameter conditions (e.g., current density, voltage, etc.). Furthermore, in some embodiments, the first and second metal oxide coatings 504, 508 can be formed by exposing the part 500 to the same electrolytic solution during the first and second anodizing processes. For example, the second anodizing process can include exposing the part 500 to the same electrolytic solution that the part 500 was previously exposed to during the first anodizing process. In other words, the part 500 does not need to be removed from the electrolytic solution in-between the first and second anodizing processes. In other embodiments, the first and second metal oxide coatings 504, 508 can be formed by exposing the part 500 to a substantially similar electrolyte. According to some examples, the electrolytic solution that is used to anodize the part 500 during the first and second anodizing processes can include one of sulfuric acid, phosphoric acid, or chromic acid.

While the first anodizing process can be performed at a relatively high current density (or voltage), such as between about 1 A/dm<sup>2</sup> to about 2 A/dm<sup>2</sup>, the second anodizing process can be performed at a lower current density (or

## 12

voltage), such as 1 A/dm<sup>2</sup> or less. In other examples, the second anodizing process can be performed at a current density between about 0.2 A/dm<sup>2</sup> to about 0.9 A/dm<sup>2</sup>. In particular, implementing a lower current density (or voltage) during the second anodizing process can impart compressive stress conditions against the part 500. Beneficially, by imparting compressive stress conditions, the second metal oxide layer 508 that is formed as a result of the second anodizing process is able to tolerate a higher level of strain, thereby significantly minimizing and/or preventing the likelihood of delamination between the oxide coating 511 and the substrate 502, as will be described in greater detail herein.

According to some embodiments, the minimized delamination and/or prevention of delamination as a result of performing the second anodizing process under reduced electrical parameter conditions (e.g., current density, voltage, etc.) can be attributed to the presence of fewer alloying agents, such as zinc, that aggregate and become enriched at an interface 520 between the substrate 502 and the second metal oxide layer 508 during the second anodizing process. Specifically, it has been found that particular alloying agents, such as zinc can combine with one or more chemical species included within the electrolytic solution to form delaminating compounds that can weaken the interfacial adhesion between the oxide coating 511 and the substrate 502 at the interface 520. In particular, the formation of delamination compounds can cause the oxide coating 511 to be susceptible to delamination (e.g., chipping, spalling, peeling, etc.), such as when the part 500 is subject to a high-impact event. In some examples, the alloying agents, such as zinc from the aluminum alloy substrate can act as an interface-weakening agent when the zinc becomes enriched at the interface 520. The zinc can aggregate at the interface 520 and form a thin layer of zinc. The enriched zinc layer can preferentially combine with sulfur-containing species, such as from a sulfuric acid electrolyte, thereby forming one or more zinc-sulfur species, such as zinc folate or a zinc sulfite. Consequently, these one or more zinc-sulfur species can act as delaminating compounds or interface-weakening agents that disrupt the interface adhesion between the oxide coating 511 and the substrate 502. However, it has been found that the enrichment of zinc at the interface 520 can be minimized and/or prevented by lowering the current density (or voltage) of the second anodizing process relative to the first anodizing process, such as 0.6 A/dm<sup>2</sup> or less. Instead zinc can become more readily incorporated directly into the second metal oxide layer 508 so as to prevent zinc from aggregating at the interface 520.

In some examples, traditionally, sulfur from the sulfuric acid electrolyte can also accumulate at the interface 520 and combine with the alloying agents so as to weaken the interface adhesion between the oxide coating 511 and the substrate 502 at the interface 520. However, by performing the second anodizing process at a relatively low current density (or voltage) can also minimize the presence of sulfur elements at the interface 520. In particular, the sulfur elements can be locked within the second metal oxide layer 508 and less driven towards the interface 520. Beneficially, this reduction of sulfur elements at the interface 520 can prevent and/or minimize zinc-sulfur compounds from interacting with the alloying agents.

According to some embodiments, the second metal oxide layer 508 formed by the techniques described herein can be characterized as having different structural properties than the first metal oxide layer 504. This difference in structural properties can be attributed to forming the second metal

oxide layer 508 under compressive stress conditions while forming the first metal oxide layer 504 under tensile strain conditions. In some examples, the pores 518 within the second metal oxide layer 508 are generally smaller in diameter than pores 505 within the first metal oxide layer 504. In some examples, the pores 518 of the second metal oxide layer 508 have pore diameters that are about half of the pore diameters of the pores 505 of the first metal oxide layer 504.

The methods described herein may be used in combination with the afore-mentioned patent publications, to yield further improvement in interfacial adhesion by a factor of two or more, without additional discoloration.

Additionally, adhesion between the oxide coating 511 and the substrate 502 can be measured using a 5-by-5 pattern of corner-linked 10 kg Vickers indents (as described in U.S. Patent publication No. 2016/0290917 A1, entitled "PROCESS FOR EVALUATION OF DELAMINATION-RESISTANCE OF HARD COATINGS ON METAL SUBSTRATES," published Oct. 6, 2016, which is incorporated by reference in its entirety for all purposes) yields fewer than 5 vertices of delamination—as compared to an unacceptable level of delamination (e.g., greater than 15 vertices of delamination) observed when the same alloy is anodized in the same electrolyte (e.g., 200 sulfuric acid) without the presently described two-step process.

Other methods identified for overcoming such interfacial adhesion problems include micro-alloying with elements such as copper and silver (as described in U.S. Patent publication No. 2017/0051426 A1, entitled "PROCESSES TO AVOID ANODIC OXIDE DELAMINATION OF ANODIZED HIGH STRENGTH ALUMINUM ALLOYS," published Feb. 23, 2017, which is incorporated by reference in its entirety for all purposes), anodizing in electrolytes comprising organic acids (such as described in U.S. Patent publication No. 2016/0060783 A1, entitled "PROCESS TO MITIGATE SPALLATION OF ANODIC OXIDE COATINGS FROM HIGH STRENGTH SUBSTRATE ALLOYS," published Mar. 3, 2016, and U.S. Patent publication No. 2016/0289858 A1, entitled "PROCESS TO MITIGATE GRAIN TEXTURE DIFFERENTIAL GROWTH RATES IN MIRROR-FINISH ANODIZED ALUMINUM," published Oct. 6, 2016, which are incorporated by reference in their entireties for all purposes). However, these methods can result in some degree of discoloration (e.g., yellowness) in the resulting oxide film.

As described above, discoloration of part 500 can be an important factor for consumer product applications. The degree of discoloration can be measured using colorimetry spectrophotometer techniques and quantified according to color space standards, such as CIE 1976 L\*a\*b\* by the International Commission on Illumination. The CIE 1976 L\*a\*b\* color space model is used to characterize colors of an object according to color opponents L\* corresponding to an amount of lightness, a\* corresponding to amounts of green and magenta, and b\* corresponding to amounts of blue and yellow. By convention, higher L\* values correspond to greater amounts of lightness and lower L\* values correspond to lesser amounts of lightness. Negative b\* values indicate a blue color, with more negative b\* values indicating a bluer color, and positive b\* values indicate a yellow color, with more positive b\* values indicating a yellower color.

Anodic oxide coatings characterized as having b\* values greater than about 1 will generally have a perceptibly yellow color. The presence of too much copper or other certain types of alloying elements within a substrate and cause part 500 to have b\* values greater than 1 when oxide coating 511

is more than about five micrometers in thickness. Since a yellow color is undesirable in some applications, in some embodiments, oxide coating 511 is characterized having a b\* value of less than 1. In some embodiments, oxide coating 511 is characterized having a b\* value between about 1 and -1 and a\* value between about 1 and -1, corresponding to a substantially colorless oxide coating 511 when undyed.

After the second anodizing process is complete, any suitable post-anodizing process can be implemented, such as an anodic film dyeing process, hydrothermal sealing process, and/or anodic film buffing/polishing process. In some applications, oxide coating 511 is left undyed and substantially colorless and hydrothermally sealed. In other applications, oxide coating 511 is colorized by depositing dye and/or metal within pores 505, and then hydrothermally sealed.

FIGS. 6A-6B show cross-section views of different portions of part 500. Part 500 can correspond to a consumer electronic device, such as device 102, 104, 106 or 108. FIG. 6A shows a portion of part 500 having a convex feature 602, such as a radius of curvature, convex edges, corner or protruding feature. FIG. 6B shows a portion of part 500 having a convex-shaped rounded feature 604, such as a rounded edge (i.e., having a curved profile), corner or protruding feature. The convex feature 602 or convex-shaped rounded feature 604 may also be small features within a textured surface, such as a blast-textured finish, a chemically etched surface, a laser-textured or laser marked finish, which exhibit roughness with features having convex radii. For simplicity, the porous structure of oxide coating 511 is not shown.

FIG. 6A shows first oxide layer 504 has channel 607 in the region over convex feature 602. Anodizing conditions of the first anodizing process combined with the tensile strain at convex feature 602 to form channel 607. As described above, the likelihood of channel 607 being formed, as well as width 608 of channel 607, will depend on conditions of the first anodizing process and the acuteness or sharpness of convex feature 602. In some embodiments, channel 607 has width 608 ranging between about 1 micrometer and about 5 micrometers. In some cases, channel 607 extends lengthwise from outer surface 516 to interface 514 between first oxide layer 504 and second oxide layer 508—i.e., through the entire thickness 506 of first oxide layer 504. In other cases, channel 607 only extends partially through the thickness 506 of first oxide layer 504.

FIG. 6B shows first oxide layer 504 has channel 617 in the region over rounded feature 604. In some embodiments, surface 601 corresponds to a bottom and generally planar surface of a bottom region of an enclosure for an electronic device, and surface 603 corresponds to a curved lateral surface (having a curved profile) of a side portion of the electronic device. Like channel 607, channel 617 was formed during the first anodizing process due, in part, to tensile strain at rounded feature 604. The likelihood of channel 617, and width 618 of channel 617, will depend on conditions of the first anodizing process and the radius of curvature of rounded feature 604. In some case, channel 617 is likely to occur when thickness 506 of first oxide layer 504 is at least 8 micrometers and the radius of curvature of rounded feature 604 is smaller than about 0.5 millimeters. In some embodiments, channel 617 has width 618 ranging between about 1 micrometer and about 5 micrometers. In some cases, channel 617 extends lengthwise from outer surface 516 to interface 514 between first oxide layer 504 and second oxide layer 508—i.e., through the entire thick-

ness **506** of first oxide layer **504**. In other cases, channel **617** only extends partially through the thickness **506** of first oxide layer **504**.

Although channels **607** and **617** extend at least partially through first oxide layer **504**, they do not penetrate through second oxide layer **508**. This is because second oxide layer **508** was formed using the second anodizing process under conditions which generate compressive stresses in the oxide film, counteracting and resisting the effective lateral growth strain induced by film growth on convex feature **602** and rounded feature **604**. In some cases, channels **607** and **617** only partially enter the second oxide layer **508**. In other cases, channels **607** and **617** terminate at interface **514** between first oxide layer **504** and second oxide layer **508**. For example, in some embodiments, second oxide layer **508** has an outer surface (defined by interface **514**) that generally conforms to the curvature of curved lateral surface **603**, while first an outer surface **516** of first oxide layer **504** has channel **617**, and therefore does not conform to the curvature of the curved lateral surface **603**. In other words, interface **514** can be characterized as having a generally constant and smooth curvature without any interruptions. In contrast, outer surface **516** of first oxide layer **504** includes channel **617**, which corresponds to an abrupt discontinuity in the curved profile of outer surface **516**. As described herein, the abrupt discontinuity in the curved profile can refer to a convex surface feature that extends from a base portion of the first oxide layer **504**.

In other cases, channels **607** and **617** penetrate through first oxide layer **504** and partially through second oxide layer **508**. In any case, channels **607** and **617** do not penetrate all the way through thickness **510** of second oxide layer **508**. In this way, second oxide layer **508** prevents channels **607** and **617** from extending to substrate **502**, thereby preventing substrate **502** from being exposed to any of a number of corrosion-inducing agents and contaminants from various environmental factors such as humidity, high temperatures, or chemicals such as salt, sweat or chlorine. These environmental exposures can be replicated and tested at accelerated rates in controlled lab environments, with salt spray testing or cycles of immersion in artificial sweat. In some cases, part **500** withstands corrosion after about 9 days of continuous salt spray testing at 65 degrees C. and 90% relative humidity (correlating to about 5 years of service in a humid marine environment).

FIG. 6C shows a cross-section view of a greater portion of part **500**. As shown, part **500** includes metal substrate **502** that is shaped and sized to form cavity **620**, which is suitable for carrying electronic components of part **500**. In this way, metal substrate **502** can serve as an enclosure. In a particular embodiment, part **500** corresponds to smart watch **106**, described above with reference to FIG. 1. Metal substrate (also referred to as an enclosure or housing) **502** includes recesses **626**, which can accept correspondingly shaped portions of a wristband so that part **500** can be worn on a user's wrist. Part **500** also includes cover **622** and component **624**, which cooperate with metal substrate **502** to complete the enclosure. In particular embodiments, cover **622** can correspond to a visibly transparent cover for a touch display assembly (not shown) that is configured to accept touch input from a user. Component **624** can include one or more light sensors configured to accept input from a user. For example, component **624** can be configured to contact a user's wrist and collect light input related to the user's heart rate. Cover **622** and component **624** can be positioned within respective openings of metal substrate **502** (i.e., within openings of metal enclosure **502**).

Oxide coating **511** covers and protects metal substrate **502** from abrasion and exposure to chemical contaminants. Oxide coating **511** can fully cover and follow the contours of metal substrate **502**, including over generally planar surface **601** of a bottom region of substrate **502** and curved lateral surface **603** of side region of substrate **502**. In some embodiments, curved lateral surface **603** has a spline-shaped curvature. For simplicity, first oxide layer **504** and second oxide layer **508** of oxide coating **511** are not depicted in FIG. 10 6C. The first oxide layer **504** of oxide coating **511** provides a cosmetically appealing and abrasion resistant outer surface for part **500**. The second oxide layer **508** of oxide coating **511** can act as a interstice-free barrier or crack-free barrier, even where portions of outer first oxide layer **504** that may have channels (e.g., **607** or **617** shown in FIGS. 6A and 6B). For example, the first oxide layer **504** portion of oxide coating **511** formed over curved side surfaces **603** and convex edges **609** may have channels from the first anodizing process. Other types of outwardly projecting features 15 of metal substrate **502** that may have oxide coating **511** with channels can include curved regions **611** proximate to recesses **626**, and bezel regions **612** proximate to cover **622**. In general, those portions of substrate **502** that are junction regions between two non-parallel sides of substrate **502** 20 (e.g., corners, curved or convex edges, protrusions, etc.) may have an oxide coating **511** with channels. The second oxide layer **508** of oxide coating **511** prevents encroachment of corrosion-inducing contaminants from reaching substrate **502** through such channels.

The corrosion-resisting oxide coatings described herein can also be used to protect features having very small dimensions. For example, FIGS. 6D and 6E show cross-section views of such small features on a textured surface **628** of part **500**, according to some embodiments. In FIG. 30 6D, shows part **500** after oxide coating **511** is formed on textured surface **628** of substrate **502**, and FIG. 6E shows part **500** after an optional oxide polishing operation is performed to smooth outer surface **516** of oxide coating **511**.

Textured surface **628** is formed by treating substrate **502** 40 with one or more surface roughening operations prior to performing the first and second anodizing processes. Suitable roughing operations can include one or more abrasive material blasting, chemical etching, laser processing, or laser-marking (e.g., if textured surface **628** corresponds to the surface of a laser-marked logo, text or other feature). Textured surface **628** is characterized as having a series of peaks **630** and valleys **632** that capture and reflect light in a way that can create matte or sparkling appearance to substrate **502**. Since peaks **630** are protrusions (i.e., have convex radii), they can cause localized in-plane tensile strain within first oxide layer **504** during the first anodizing process, and therefore can cause channel **634** to form. Of course, more than one channel **634** can be formed within first oxide layer **504**, the prevalence of which will depend on 45 the size of peaks **630**, as well as the conditions of the first anodizing process. In some embodiments, peaks **630** having heights **636** of about 5 micrometers or more may cause channel **634** to form using some Type II anodizing processes. In any case, second oxide layer **508**, formed using the compressive stress second anodizing process, prevents channel **634** from extending to substrate **502** and thereby 50 protects substrate **502** from exposure to corrosion-inducing agents or other contaminants.

It should be noted that the surface features that can cause 55 sufficient in-plane tensile strain to cause cracks or channels to form during anodizing are not limited to the examples described above. That is, any protruding, outwardly curved,

convex-shaped, convex edges or corner surface features may be associated with forming a channel within the first oxide layer. Other examples may include metal surfaces of buttons (e.g., watch crown), switches, bezels, frames, brackets other suitable components of electronic devices. The channels within the first oxide layer may be positioned proximate to the surface features, such as above the surface feature (with the second oxide layer positioned between the first oxide layer and a metal surface of the underlying substrate).

FIGS. 7A and 7B show scanning electron microscope (SEM) images of cross-sections views of a part having a corrosion-resisting oxide coating, with FIG. 7B showing a higher magnification SEM image. The part in FIGS. 7A and 7B includes aluminum alloy substrate 702 having edge 703, which has an oxide coating with first oxide layer 704 (also referred to as an outer oxide layer) formed using a first anodizing process and second oxide layer 708 (also referred to as an inner oxide layer) formed using a compressive stress second anodizing process, as described above. As shown, channel 707 formed during the first anodizing process extends at least partially through the thickness of first oxide layer 704 but does not extend through second oxide layer 708, thereby preventing contaminant from reaching substrate 702. This is because second oxide layer 708 is formed under compressive stress conditions that prevent channel 707 from forming within or extending through second oxide layer 708.

FIG. 8 illustrates flowchart 800, indicating a process for forming a corrosion-resisting oxide coating on a part, in accordance with some embodiments. At 802, a protruding feature is formed on a substrate, such as an aluminum or an aluminum alloy substrate. The protruding feature can correspond to an edge, corner or other outwardly extending feature. The protruding feature can have a curved profile or an angular profile. In a particular embodiment, protruding feature corresponds to a curved edge or corner of an enclosure for an electronic device. The feature can be formed using any suitable technique, including a machining operation, etching operation, molding operation, or suitable combination thereof. It may even be formed by a surface 40 texturing operation such as blasting, chemical etching, laser processing, or laser-marking of a logo or text.

At 804, the substrate is optionally treated prior to an anodizing process. Suitable pretreatments can include etching, polishing and/or abrasive blasting the surface of the 45 substrate that is to be anodized. In some cases the surface of the substrate is polished to achieve a target gloss value. At 806, a first oxide layer of an oxide coating is formed on the substrate using a first anodizing process. In some applications, the first anodizing process is a Type II anodizing process using an aqueous sulfuric acid electrolyte. The first anodizing process can form a relatively hard first oxide layer (e.g., having a hardness value of at least 350 HV<sub>0.05</sub>); however, these conditions can cause one or more cracks or channels to form within the first oxide layer over the 55 protruding feature.

At 808, a second oxide layer of the oxide coating is formed adjacent the substrate using a second anodizing process. The second anodizing process is performed under compressive stress conditions, which can involve anodizing using a low current density (e.g., 0.8 A/dm<sup>-2</sup>), low voltage, or high electrolyte temperature. The compressive stress conditions result in the second oxide layer to be softer than the first oxide layer, but also less likely to develop a channel, even over the protruding feature. Thus, the second oxide layer acts as a barrier between the outer environment and the substrate, thereby protecting the substrate from exposure to

corrosion-inducing agents. The thickness of the second oxide layer is thin (e.g., between about 0.5 and 2 micrometers) such that the majority thickness of the oxide coating is formed under process conditions which yield a relatively 5 hard coating.

At 810, the oxide coating is optionally colored using one or more coloring processes. In some embodiments, this involves depositing a dye and/or metal material within pores of the oxide coating. In other embodiments, the coloring process is skipped such that the oxide coating is substantially colorless. At 812, the oxide coating is optionally sealed using, for example, a hydrothermal sealing process that closes the pores within the oxide coating, thereby further increasing the corrosion-resisting properties of the oxide coating. At 814, the oxide coating is optionally polished using, for example, one or more buffing, lapping or other polishing operations to provide a shine to an exterior surface to the oxide coating.

The foregoing description, for purposes of explanation, uses specific nomenclature to provide a thorough understanding of the described embodiments. However, it will be apparent to one skilled in the art that the specific details are not required in order to practice the described embodiments. Thus, the foregoing descriptions of the specific embodiments described herein are presented for purposes of illustration and description. They are not intended to be exhaustive or to limit the embodiments to the precise forms disclosed. It will be apparent to one of ordinary skill in the art that many modifications and variations are possible in view of the above teachings.

What is claimed is:

1. A part, comprising:  
an enclosure of a portable electronic device;  
a metal substrate defining a curved surface; and  
a metal oxide coating disposed on the metal substrate at  
the curved surface, the metal oxide coating comprising:  
a first porous oxide layer defining an interstice extending  
through the first porous oxide layer; and  
a second porous oxide layer disposed between the first  
porous oxide layer and the metal substrate, the  
second porous oxide layer defining a barrier between  
the metal substrate and an ambient environment at  
the interstice.

2. The part of claim 1, wherein the first porous oxide layer has a first set of pore structures having a first diameter, and the second porous oxide layer has a second set of pore structures having a second diameter that is less than the first diameter.

3. The part of claim 1, wherein:  
an interface separates the second porous oxide layer from  
the metal substrate, the interface and second porous  
metal oxide layer comprising sulfur elements; and  
fewer sulfur elements are disposed at the interface than  
within the second porous oxide layer.

4. The part of claim 1, wherein a thickness of the second porous oxide layer is between about 0.2 micrometer and about 2 micrometers, and a thickness of the first porous oxide layer is between about 10 micrometers and about 20 micrometers.

5. The part of claim 1, wherein the metal oxide coating has a Vickers hardness of at least about 300 HV<sub>0.05</sub> or greater.

6. The part of claim 1, wherein the curved surface has a 65 radius of curvature of less than 0.5 mm.

7. The part of claim 1, wherein the second porous oxide layer is under a compressive stress.

19

8. A process for anodizing a metal substrate comprising an enclosure of a portable electronic device having a convex surface geometry, the process comprising disposing a metal oxide coating on the convex surface comprising:  
 converting a first amount of the metal substrate to a first porous metal oxide layer under a tensile strain condition that corresponds to a first electrical parameter, wherein the first porous metal oxide layer defines an interstice extending through the first porous metal oxide layer; and  
 converting a second amount of the metal substrate that is overlaid by the first porous metal oxide layer to a second porous metal oxide layer under a compressive stress condition that corresponds to a second electrical parameter, the second porous metal oxide layer being positioned between the first porous metal oxide layer and a remaining portion of the metal substrate, the second porous metal oxide layer defining a barrier that separates the interstice from the metal substrate.
9. The process of claim 8, wherein the first and second amounts of the metal substrate are converted to the first and second porous metal oxide layers using a same electrolyte.
10. The process of claim 8, wherein the first electrical parameter is greater than the second electrical parameter, and the first and second electrical parameters comprise a first current density and a second current density or a first voltage and a second voltage.
11. The process of claim 10, wherein the first current density is between about  $1.0 \text{ A/dm}^{-2}$  and about  $2.0 \text{ A/dm}^{-2}$ , and the second current density is no greater than about  $0.8 \text{ A/dm}^{-2}$ .
12. The process of claim 8, wherein a thickness of the second porous metal oxide layer is no greater than about 2 micrometers.
13. The process of claim 8, wherein converting the second amount of the metal substrate to the second porous metal oxide layer under the compressive stress condition limits

20

- alloying agents from aggregating at an interface between the second porous metal oxide layer and the metal substrate.
14. A method for forming a metal oxide layer on a curved surface of a metal substrate comprising an enclosure of a portable electronic device, the metal oxide layer comprising an inner porous oxide layer and an outer porous oxide layer disposed on the inner porous oxide layer, the method comprising:  
 forming the outer porous oxide layer by exposing a first portion of the metal substrate to an electrolyte under a tensile strain condition that corresponds to a first current density, the outer porous oxide layer defining an interstice extending through the outer porous oxide layer; and  
 forming the inner porous oxide layer by exposing a second portion of the metal substrate to the electrolyte under a compressive stress condition that corresponds to a second current density that is less than the first current density, the inner porous oxide layer defining a barrier between the metal substrate and an ambient environment.
15. The method of claim 14, wherein the first current density is about  $1.0 \text{ A/dm}^{-2}$  or greater and the second current density is about  $0.6 \text{ A/dm}^{-2}$  or less.
16. The method of claim 14, wherein the metal oxide layer has a Vickers hardness of at least about  $300 \text{ HV}_{0.05}$  or greater.
17. The method of claim 14, wherein the inner porous oxide layer has a thickness between about 0.2 micrometers and about 2 micrometers, and the inner porous oxide layer defines pore structures with pore diameters that are about half of pore diameters of pore structures defined by the outer porous oxide layer.
18. The method of claim 14, wherein the metal oxide layer has fewer than 5 vertices of delamination as measured according to a 5-by-5 pattern of corner-linked 10 kg Vickers indents.

\* \* \* \* \*